

1

3,473,948

**METHOD OF IMPROVING RESIN FINISHED  
TEXTILES**

John Dean Turner, Greensboro, N.C., assignor to  
Burlington Industries, Inc., Greensboro, N.C., a  
corporation of Delaware  
No Drawing. Filed Sept. 29, 1966, Ser. No. 583,062  
Int. Cl. B44d 1/20, 1/44

U.S. Cl. 117—62.1

8 Claims

**ABSTRACT OF THE DISCLOSURE**

Process for improving the properties of resin-treated cellulosic textiles by hydrolyzing the resin-treated textile in an aqueous bath containing a strong acid and an alkali metal, alkaline earth metal or ammonium salt electrolyte and then neutralizing and washing the hydrolyzed textile. The resulting product is characterized by improved abrasion resistance.

This invention relates to improved resin-finished textiles and the method of making the same. More specifically it relates to resin-finished textile materials with improved abrasion resistance and the method of making the same.

**BACKGROUND OF THE INVENTION**

Cellulose fiber-containing textiles such as cotton, rayon, linen and blends of these fibers have long been used in making garments. In recent years a number of various methods have been developed for treating such textile fabrics to impart desirable crease resistance, and also to impart "permanent press" characteristics to the textile fabrics. The majority of these methods involve the use of thermosetting resins. The use of thermosetting resin-finished textiles containing cellulosic fibers, such as cotton, regenerated cellulose (rayon) and blends thereof with other natural and/or synthetic fibers, has become much more widespread.

Typical patents relating to resin-finished cellulosic textiles are Hurwitz, U.S. Patent 2,950,553; Warnock et al., U.S. Patent 2,974,432 and Getchell, U.S. Patent 3,166,765, the disclosures of which are hereby incorporated by reference.

The copending application of Tomasino and Smith, application No. 521,443, filed Jan. 18, 1966 and assigned to the assignee of the present invention, is likewise directed to a process for resin-finishing cellulosic textile with curable resins or reactants for the purpose of obtaining durable finish or surface effects. The disclosure of this application is also incorporated herein by reference.

**OBJECTS OF THE INVENTION**

It is an object of this invention to provide novel, improved resin-finished cellulosic textiles. It is a further object of the invention to provide resin-finished cellulosic textiles with improved abrasion resistance. It is another object of this invention to provide resin-finished cellulosic textiles with improved abrasion resistance, tear strength, handle, moisture regain and soil resistance. Yet another object of this invention is to provide a process for the production of resin-finished cellulosic textiles with improved abrasion resistance. A further object of this invention is to provide a process for the production of resin-finished cellulosic textiles with improved abrasion resistance, tear strength, handle, moisture regain and soil resistance.

Still further objects and the entire scope of applicability of the present invention will become apparent from the detailed description given hereinafter; it should be understood, however, that the detailed description and specific examples, while indicating preferred embodiments of the invention, are given by way of illustration only, since various changes or modifications within the scope of the

2

invention will become apparent to those skilled in the art from this detailed description.

**SUMMARY OF THE INVENTION**

Improved resin-finished cellulosic textiles with increased abrasion resistance are produced by (a) subjecting resin-treated textiles, which have been treated with a cross-linking agent and at least partially cured, to a hydrolyzing step in an aqueous bath with a strong organic or mineral acid in the presence of an alkali metal, alkaline earth metal, or ammonium salt electrolyte and (b) immediately thereafter neutralizing the fabric.

**DESCRIPTION OF THE INVENTION**

The present invention resides in the process of subjecting a resin-treated textile, which is at least partially cured, to a hydrolyzing step by immersing the textile in an aqueous bath containing a strong organic or mineral acid and also containing an alkali metal salt electrolyte, an alkaline earth metal salt electrolyte, or an ammonium salt electrolyte, and thereafter neutralizing and washing the textile.

Suitable cellulosic or cellulose-containing textiles were described above and include, but are not to be limited to, cotton, rayon, linen and blends of these fibers with other natural and synthetic fibers. The present invention contemplates a fabric containing at least 20 percent of cellulosic fibers.

Suitable resins for cross-linking agents were described above. Any of the conventional curing resins or reactants which are used for the treatment of cellulosic textiles to give durable surface effects, e.g., permanent press, wash-wear or the like, may be used herein. This includes, for example, the methyloinated derivatives of various nitrogen-containing compounds such as urea, N,N'-ethylene urea, propylene urea, aminotriazines such as melamines and substituted melamines, triazines and urons. Combinations of these materials, for example, a mixture of polymethylolated triazine and polymethylolated ethylene urea, may also be employed.

The amount of reactant or resin which is applied to the fabric according to the invention may be widely varied and will depend on other operating factors, e.g., the fabric construction, reactant employed and the properties described in the ultimate product. However, the amount will generally be in the range of about 2-20% solids add-on based on the weight of the fabric although amounts outside this range may also be employed.

The resin and the cross-linking agent are applied in the usual manner and at least partially cured prior to the hydrolyzing step.

The hydrolysis may be conducted as either a continuous process or a batch process with the fabric in open width or in rope form. The hydrolyzing bath may contain 0.01 to 15% w/v. of the acid, and preferably 2 to 5% w/v. of the acid; and from 5% w/v. up to the saturation point of the electrolyte salt, and preferably 15 to 25% w/v. of the electrolyte salt.

The hydrolyzing acid is a strong organic or mineral acid. Typical examples, which should not be construed to limit the invention thereto, of such an acid are hydrochloric acid, nitric acid, chloric acid, hydrobromic acid, hydroiodic acid, perchloric acid, sulfuric acid, trichloroacetic acid, dichloroacetic acid, monobromoacetic acid, alpha-chloropropionic acid, malonic acid, formic acid, oxalic acid, thiocyanoacetic acid, lactic acid and cyanoacetic acid.

The term "electrolyte" is defined by the Condensed Chemical Dictionary, 6th edition, as "a substance which dissociates into ions when in a solution or a fused state and it will then conduct an electric current." This invention contemplates the use of electrolytes which are salts of alkali metals, alkaline earth metals, or ammonium

salts. Suitable salts for the present invention, for example, include sodium chloride, sodium hydrogen phosphates, sodium nitrate, potassium chloride, sodium sulphate, calcium chloride, magnesium chloride, ammonium chloride, potassium nitrate, potassium ferricyanide, potassium bromide, etc. The above listing is by way of exemplification only and is not to be construed to limit the present invention in any way.

After the hydrolysis step, the textile fabric is immediately neutralized and washed. The preferred neutralizing agent is a weak alkaline compound, for example, ammonia, sodium carbonate or sodium bicarbonate. The neutralization may be accomplished by a variety of ways, such as immersing the fabric in a neutralizing bath, spraying the fabric with a solution of the neutralizing compound, subjecting the fabric to the action of vapors of the neutralizing agent, etc. The preferred method of neutralization is by immersing the fabric in a bath containing the neutralizing agent. The bath temperature may vary over a wide temperature range, i.e. 40° F.-180° F., but preferably is approximately room temperature. The bath concentration and temperature and the duration of the treatment determine the degree of acid neutralization. Preferably, the duration of the treatment will be of ½ to 2 minutes although the treatment time may vary from ¼ to 30 minutes in length. Generally, treatment times of over 5 minutes may be used but are not practical from an economic standpoint. The bath concentration may vary from quite weak, e.g., ¼% w/v., up to quite concentrated solutions, e.g., 15% w/v. The neutralization bath preferably contains about 5 to 10% w/v. of the neutralizing agent.

After the neutralization, the fabric is preferably washed with water to remove any residual traces of neutralizing agent or neutralizing acid. Any of the conventional washing operations commonly used in the textile art may be utilized, e.g., immersion or spraying.

In the production of certain resin-finished cellulose textiles, depending upon the particular resin, cross-linking agents, and cellulosic textile involved, it may be advantageous to incorporate minor amounts—e.g., 0.001 to 3% w/v.—of a wetting agent. Almost any conventional wetting agent commonly used in the textile art may be utilized, for example, adducts of sorbitol and propylene oxide or ethylene oxide.

One of the common techniques known to the art for improving the abrasion resistance of cellulose textiles has been the application of a film-forming additive and/or lubricating agent to the textile. Such materials may be added before and/or after the hydrolyzing step of the present invention, and the resulting resin-finished cellulose textile generally has abrasion resistance exceeding that produced by either step alone. Acrylic resins have been commonly used as such film-forming additives and lanolin-based lubricating agents, such as Bi-Chem Softener LLS,

which is a mixture of lanolin and polyethylene emulsions, may be used as the lubricating agent. Preferably the acrylic resin is used before and after the acid hydrolysis step.

The temperature and the time of the hydrolysis will depend upon the particular fabric involved and the results desired. Generally, temperatures in the order of 70 to 210° F. may be used and more preferably temperatures of 100 to 200° F. may be used. Generally, times in excess of five minutes are uneconomical and times less than one-fourth of a minute do not allow sufficient hydrolyzation to occur. Therefore, the time of the hydrolyzing step will generally be from one-fourth to five minutes, and most preferably from one-half to three minutes.

The hydrolyzing step process of the present invention readily lends itself to the production of fibers which may be permanently pleated or shaped. The cellulose textile may be treated with the resin and the cross-linking agent, and partially cured. The partially cured fabric is then hydrolyzed to produce a resin-finished cellulose textile with improved abrasion resistance which may be subsequently permanently pleated or shaped.

Other properties of the resin-treated cellulose textiles of this invention are improved in addition to the abrasion resistance. For example, tear strength, handle, moisture regain and soil resistance generally show a marked improvement as compared to ordinarily treated cellulose textiles.

Although any alkali metal salt, alkaline earth metal salt, or ammonium salt electrolyte may be used according to the present invention, preferred salts are those of the hydrolyzing acid utilized. Most preferably, the hydrolyzing acid is hydrochloric acid and the electrolyte salt is sodium chloride. It is necessary that the electrolyte salts be neutral or slightly acid. Buffering compounds, such as sodium carbonate, should be avoided. The electrolyte salt cation will be an alkali metal cation, an alkaline earth metal cation, or an ammonium cation, while the electrolyte salt anion will be a strong organic acid or mineral acid anion, and preferably is the anion corresponding to the anion of the hydrolyzing acid.

The resin-treated cellulose fabric may optionally be pre-wetted before the hydrolyzing step. The pre-wetting may, for example, be effected by passing the fabric through an aqueous bath which may optionally contain minor amounts of a conventional wetting agent.

When used in this specification, the expression "% w/v." means weight percent by volume, that is, weight percent based on the total volume of solution, and W and F represent warp and fill, respectively.

In the following examples, the resin-treated fabric was passed through a first aqueous bath containing the hydrochloric acid and the sodium chloride, then through a neutralizing aqueous bath containing 2% w/v. of sodium carbonate, and thereafter through an aqueous washing bath, and dried at 120° F.

TABLE 1

Fabric: 100% Cotton, Army Twill; Treatment: 30% Resin 183,<sup>1</sup> 6% Catalyst 43,<sup>2</sup> Dry at 200° F. for 3 minutes; Cure at 340° F. for 6 minutes.

|                                        | Example |         |         |         |         |
|----------------------------------------|---------|---------|---------|---------|---------|
|                                        | 1       | 2       | 3       | 4       | 5       |
| NaCl <sup>3</sup>                      | 0       | 0       | 30      | 30      | 0       |
| HCl <sup>4</sup>                       | 0.5     | 0.5     | 0.5     | 0.5     | 0       |
| Temp., °F.                             | 140     | 140     | 140     | 140     | 140     |
| Time (min.)                            | 2       | 5       | 2       | 5       | 0       |
| Tear Strength (W/F)                    | 1.5/0.9 | 1.5/1.1 | 1.8/1.5 | 1.8/1.4 | 1.4/0.9 |
| Crease Resistance (W+F), Dry           | 256     | 254     | 248     | 244     | 261     |
| Crease Resistance (W+F), Wet           | 283     | 277     | 274     | 275     | 277     |
| Stoll Flex Abrasion, <sup>5</sup> Warp | 41      | 67      | 144     | 120     | 46      |
| Stoll Flex Abrasion, <sup>5</sup> Fill | 269     | 300     | 504     | 490     | 235     |
| Weight (oz./sq. yd.)                   | 8.28    | 8.28    | 8.38    | 8.20    | 8.33    |
| Edge Abrasion:                         |         |         |         |         |         |
| 5 min.                                 | 4       | 4       | 5       | 5       | 4       |
| 7 min.                                 | 3       | 3       | 4       | 4       | 3       |
| 9 min.                                 | 2       | 1       | 3       | 4       | 3       |

<sup>1</sup> Dihydroxydimethylol ethylene urea, by Sun Chemical Company.

<sup>2</sup> Zinc nitrate solution, by Bi-Chem, Burlington Industries, Inc.

<sup>3</sup> Concentrations are defined as grams per liter, e.g., 30% means 300 grams of reagent per liter.

<sup>4</sup> Concentrated hydrochloric acid, approximately 37%.

<sup>5</sup> ½ lb. head load, 2 lbs. tension.

TABLE 2

Fabric: 75% Cotton/25% Polyester Twill; Pretreatment: 30% Resin 183, 6% Catalyst, Dry 3 minutes at 200° F.; Cure 6 minutes at 340° F.

|                              | Example |         |         |         |  |
|------------------------------|---------|---------|---------|---------|--|
|                              | 6       | 7       | 8       | 9       |  |
| NaCl                         | 25      | 25      | (1)     | (2)     |  |
| HCl                          | 0.5     | 0.5     | (1)     | (2)     |  |
| Temp., ° F.                  | 140     | 140     | (1)     | (2)     |  |
| Time (min.)                  | 5       | 15      | (1)     | (2)     |  |
| Tear Strength (W/F)          | 1.9/2.2 | 1.6/1.6 | 1.9/1.9 | 3.4/4.5 |  |
| Crease Resistance (W+F), Dry | 263     | 270     | 277     | 179     |  |
| Crease Resistance (W+F), Wet | 272     | 281     | 283     | 198     |  |
| Stoll-Flex Abrasion, Warp    | 1,500   | 518     | 451     | 1,246   |  |
| Stoll-Flex Abrasion, Fill    | 1,500   | 1,120   | 1,021   | 1,500   |  |
| Weight (oz./sq. yd.)         | 7.90    | 8.33    | 7.94    | 7.54    |  |

<sup>1</sup> Resin treated, but no hydrolysis.

<sup>2</sup> Control, no resin no hydrolysis.

TABLE 3

Fabric: 100% Cotton, Army Twill; Pretreatment: 25% Bi-Chem HK, <sup>1</sup> Dry 3 minutes at 200° F.; 5% Catalyst 43, Cure 6 minutes at 340° F.

|                              | Example |         |         |         |         |
|------------------------------|---------|---------|---------|---------|---------|
|                              | 10      | 11      | 12      | 13      | 14      |
| NaCl                         | 15      | 20      | 25      | 15      | 20      |
| HCl                          | 0.5     | 0.5     | 0.5     | 0.5     | 0.5     |
| Temp., ° F.                  | 140     | 140     | 140     | 140     | 140     |
| Time (min.)                  | 3       | 3       | 3       | 5       | 5       |
| Tear Strength (W/F)          | 1.8/1.4 | 2.6/2.4 | 1.6/1.3 | 1.8/1.5 | 1.8/1.6 |
| Crease Resistance (W+F), Dry | 248     | 290     | 252     | 221     | 212     |
| Crease Resistance (W+F), Wet | 267     | 285     | 273     | 258     | 264     |
| Stoll-Flex Abrasion, Warp    | 118     | 376     | 91      | 132     | 155     |
| Stoll-Flex Abrasion, Fill    | 419     | 545     | 333     | 629     | 360     |
| Weight (oz./sq. yd.)         | 8.50    | 8.53    | 8.37    | 8.31    | 8.33    |

<sup>1</sup> Dihydroxydimethylol ethylene urea, by Bi-Chem, Burlington Industries, Inc.

TABLE 4.—EFFECT OF PREWETTING BEFORE HYDROLYSIS

Fabric: 100% Cotton, Army Twill; Pretreatment: 25% Resin 183, 5% Catalyst 43, Dry at 250° F. for 3 minutes; Cure at 340° F. for 6 minutes.

|                                   | Example |         |         |         |         |         |         |       |
|-----------------------------------|---------|---------|---------|---------|---------|---------|---------|-------|
|                                   | 15      | 16      | 17      | 18      | 19      | 20      | 21      | 22    |
| Prewet before hydrolysis          | Yes     | No      | Yes     | No      | Yes     | No      | X       | X     |
| NaCl                              | 15      | 15      | 20      | 20      | 25      | 25      | X       | X     |
| HCl                               | 0.5     | 0.5     | 0.5     | 0.5     | 0.5     | 0.5     | X       | X     |
| Temp., ° F.                       | 140     | 140     | 140     | 140     | 140     | 140     | X       | X     |
| Time (min.)                       | 2       | 2       | 2       | 2       | 2       | 2       | X       | X     |
| After treatment:                  |         |         |         |         |         |         | X       | X     |
| K-3 Acrylic <sup>1</sup>          | 4       | 4       | 4       | 4       | 4       | 4       | 4       | 4     |
| Bi-Chem Softener LLS <sup>2</sup> | 2       | 2       | 2       | 2       | 2       | 2       | X       | 2     |
| Catalyst 43                       | 0.5     | 0.5     | 0.5     | 0.5     | 0.5     | 0.5     | X       | 0.5   |
| Tear Strength (W/F)               | 2.2/1.8 | 2.0/1.7 | 4.0/1.6 | 2.3/2.0 | 2.2/1.8 | 2.3/1.7 | 1.5/1.0 | 1.8/2 |
| Crease Resistance:                |         |         |         |         |         |         |         |       |
| (W+F), Dry                        | 319     | 306     | 311     | 311     | 321     | 326     | 286     | 29.9  |
| (W+F), Wet                        | 299     | 298     | 300     | 302     | 317     | 313     | 280     | 297   |
| Stoll-Flex Abrasion:              |         |         |         |         |         |         |         |       |
| Warp                              | 118     | 78      | 83      | 201     | 105     | 132     | 49      | 66    |
| Fill                              | 638     | 446     | 401     | 455     | 729     | 486     | 265     | 352   |
| Weight (oz. sq. yd.)              | 8.46    | 8.50    | 8.48    | 8.52    | 8.53    | 8.70    | 8.53    | 8.64  |

<sup>1</sup> Rohm and Haas, Rhoplex K-3 acrylic (U.S. Pat. 3,157,562).

<sup>2</sup> Bi-Chem, Burlington Industries, Inc., Lanolin Base.

TABLE 5

Fabric: 100% All Cotton, Yard Stick (Mooresville Fabric); Pretreatment: 25% Resin 183, 4.5% Catalyst 43, Dry at 250° F. for 3 minutes; Cure at 320° F. for 10 minutes.

|                      | Example |      |      |      |      |      |      |      |      |  |
|----------------------|---------|------|------|------|------|------|------|------|------|--|
|                      | 23      | 24   | 25   | 26   | 27   | 28   | 29   | 30   | 31   |  |
| NaCl                 | 20      | 20   | 20   | 20   | 25   | 25   | 25   | 25   | X    |  |
| HCl                  | 0.5     | 0.5  | 0.5  | 0.5  | 0.5  | 0.5  | 0.5  | 0.5  | X    |  |
| Temp., ° F.          | 140     | 140  | 170  | 170  | 140  | 140  | 170  | 170  | X    |  |
| Time (min.)          | 1       | 2    | 1    | 2    | 1    | 2    | 1    | 2    | X    |  |
| After treatment:     |         |      |      |      |      |      |      |      |      |  |
| K-3 Acrylic          | 4       | 4    | 4    | 4    | 4    | 4    | 4    | 4    | 4    |  |
| Bi-Chem softener LLS | 2       | 2    | 2    | 2    | 2    | 2    | 2    | 2    | 2    |  |
| Catalyst 43          | 1       | 1    | 1    | 1    | 1    | 1    | 1    | 1    | 1    |  |
| Tear Strength:       |         |      |      |      |      |      |      |      |      |  |
| Warp                 | 1.4     | 1.8  | 1.9  | 1.7  | 1.9  | 2.1  | 1.8  | 1.8  | 1.2  |  |
| Fill                 | 0.7     | 0.8  | 7.7  | 8.5  | 7.2  | 0.7  | 0.7  | 0.8  | 0.6  |  |
| Crease Resistance:   |         |      |      |      |      |      |      |      |      |  |
| (W+F), Dry           | 318     | 317  | 316  | 306  | 309  | 315  | 316  | 304  | 320  |  |
| (W+F), Wet           | 289     | 291  | 298  | 277  | 278  | 287  | 296  | 283  | 271  |  |
| Stoll-Flex Abrasion: |         |      |      |      |      |      |      |      |      |  |
| Warp                 | 14      | 26   | 30   | 35   | 44   | 117  | 20   | 32   | 13   |  |
| Fill                 | 6       | 10   | 10   | 22   | 18   | 23   | 8    | 12   | 6    |  |
| Weight (oz./sq. yd.) | 3.38    | 3.38 | 3.35 | 3.39 | 3.33 | 3.40 | 3.35 | 3.32 | 3.39 |  |

TABLE 6

Fabric: 100% Cotton, Army Twill; Pretreatment: As Indicated. Dry 3 minutes at 200° F., Cure 10 minutes at 320° F.

|                      | Example |      |      |      |      |      |      |       |
|----------------------|---------|------|------|------|------|------|------|-------|
|                      | 32      | 33   | 34   | 35   | 36   | 37   | 39   | 38    |
| Resin                | 15      | 15   | 20   | 20   | 25   | 25   | 25   | 25    |
| Catalyst 43          | 2.7     | 2.7  | 3.6  | 3.6  | 4.5  | 4.5  | 4.5  | 4.5   |
| NaCl                 | 20      | 20   | 20   | 20   | 20   | 20   | 20   | 20    |
| HCl                  | 0.5     | 0.5  | 0.5  | 0.5  | 0.25 | 1    | 2    | 3     |
| Temp., ° F           | 140     | 140  | 140  | 140  | 140  | 140  | 140  | 140   |
| Time (min.)          | 2       | 2    | 2    | 2    | 2    | 2    | 2    | 2     |
| Aftertreatment:      |         |      |      |      |      |      |      |       |
| K-3 Acrylic          | 4       | X    | 4    | X    | 4    | 4    | 4    | 4     |
| Bi-Chem Softener LLS | 2       | X    | 2    | X    | 2    | 2    | 2    | 2     |
| Catalyst 43          | 0.5     | X    | 0.5  | X    | 0.5  | 0.5  | 0.5  | 0.5   |
| Tear Strength:       |         |      |      |      |      |      |      |       |
| Warp                 | 2.8     | 1.8  | 2.0  | 2.4  | 3.7  | 3.5  | 3.7  | 3.9   |
| Fill                 | 2.4     | 1.6  | 1.8  | 2.6  | 2.8  | 3.2  | 2.9  | 3.6   |
| Crease Resistance:   |         |      |      |      |      |      |      |       |
| (W+F), Dry           | 306     | 248  | 303  | 245  | 311  | 309  | 307  | 288   |
| (W+F), Wet           | 286     | 270  | 292  | 269  | 301  | 304  | 299  | 302   |
| Stoll Flex Abrasion: |         |      |      |      |      |      |      |       |
| Warp                 | 240     | 110  | 116  | 110  | 160  | 199  | 325  | 512   |
| Fill                 | 1,125   | 389  | 647  | 363  | 688  | 737  | 727  | 1,218 |
| Weight (oz./sq. yd.) | 8.14    | 8.08 | 8.32 | 8.32 | 8.32 | 8.30 | 8.31 | 8.26  |

TABLE 7

Fabric: 100% Cotton, Yarn Stick; Pretreatment: 25% Resin 183, 4.5% Catalyst 43, Dry at 200° F. for 3 minutes; Cure at 320° F. for 10 minutes.

|                      | Example |         |         |         |         |
|----------------------|---------|---------|---------|---------|---------|
|                      | 40      | 41      | 42      | 43      | 44      |
| NaCl                 | X       | 20      | 20      | 25      | 25      |
| HCl                  | X       | 0.5     | 0.5     | 0.5     | 0.5     |
| Temp., ° F           | X       | 200     | 200     | 200     | 200     |
| Time (min.)          | X       | ½       | 1       | ½       | 1       |
| Aftertreatment:      |         |         |         |         |         |
| K-3 Acrylic          | 4       | 4       | 4       | 4       | 4       |
| Bi-Chem Softener LLS | 2       | 2       | 2       | 2       | 2       |
| Catalyst 43          | ½       | ½       | ½       | ½       | ½       |
| Tear Strength (W/F)  | 1.1/0.5 | 1.8/8.5 | 1.7/0.8 | 1.9/0.8 | 1.8/0.9 |
| Crease Resistance:   |         |         |         |         |         |
| (W+F), Dry           | 323     | 309     | 301     | 285     | 290     |
| (W+F), Wet           | 292     | 287     | 299     | 263     | 283     |
| Stoll Flex Abrasion: |         |         |         |         |         |
| Warp                 | 16      | 27      | 50      | 74      | 52      |
| Fill                 | 8       | 17      | 22      | 61      | 31      |
| Weight (oz./sq. yd.) | 3.38    | 3.38    | 3.39    | 3.38    | 3.38    |

TABLE 8

Fabric: 100% Cotton, Army Twill; Pretreatment: 25% Resin 183, 4.5% Catalyst 43, 4% Rhoplex K-3, Dry at 200° F. for 3 minutes; Cure at 320° F. for 10 minutes.

|                      | Example |      |      |      |      |      |      |
|----------------------|---------|------|------|------|------|------|------|
|                      | 45      | 46   | 47   | 48   | 49   | 50   | 51   |
| NaCl                 | 15      | 15   | 20   | 20   | 20   | 20   | X    |
| HCl                  | 5       | 5    | 0.5  | 0.5  | 0.5  | 0.5  | X    |
| Temp., ° F           | 140     | 140  | 170  | 170  | 170  | 170  | X    |
| Time (min.)          | 3       | 3    | 1    | 1    | 2    | 2    | X    |
| Aftertreatment:      |         |      |      |      |      |      |      |
| Rhoplex K-3          | 4       | X    | 4    | X    | 4    | X    | 4    |
| Bi-Chem Softener LLS | 2       | X    | 2    | X    | 2    | X    | 2    |
| Catalyst 43          | ½       | X    | ½    | X    | ½    | X    | ½    |
| Tear Strength:       |         |      |      |      |      |      |      |
| Warp                 | 3.2     | 2.0  | 2.2  | 1.7  | 2.3  | 2.0  | 1.9  |
| Fill                 | 2.8     | 2.0  | 1.9  | 1.5  | 2.1  | 1.8  | 1.5  |
| Crease Resistance:   |         |      |      |      |      |      |      |
| (W+F), Dry           | 291     | 287  | 322  | 317  | 318  | 310  | 321  |
| (W+F), Wet           | 302     | 294  | 306  | 294  | 303  | 301  | 305  |
| Stoll Flex Abrasion: |         |      |      |      |      |      |      |
| Warp                 | 1,261   | 281  | 202  | 145  | 277  | 189  | 80   |
| Fill                 | 1,870   | 966  | 696  | 359  | 962  | 416  | 491  |
| Weight (oz./sq. yd.) | 8.46    | 8.33 | 8.43 | 8.36 | 8.48 | 8.46 | 8.41 |

TABLE 9

Fabric: 100% Cotton Broadcloth; Pretreatment: 25% Resin HK, 4.5% Catalyst 43, Dry at 200° F. for 3 minutes; Cure at 320° F. for 10 minutes.

|                      | Example |     |     |     |     |     |     |     |
|----------------------|---------|-----|-----|-----|-----|-----|-----|-----|
|                      | 53      | 54  | 55  | 56  | 57  | 58  | 59  | 60  |
| NaCl                 | 25      | 25  | 25  | 25  | 20  | 20  | 20  | 20  |
| HCl                  | 3       | 3   | 3   | 3   | 3   | 3   | 3   | 3   |
| Temp., ° F           | 140     | 140 | 140 | 140 | 140 | 140 | 140 | 140 |
| Time (min.)          | 1       | 2   | 3   | 5   | 1   | 2   | 3   | 5   |
| Aftertreatment:      |         |     |     |     |     |     |     |     |
| Rhoplex K-3          | 3       | 3   | 3   | 3   | 3   | 3   | 3   | 3   |
| Bi-Chem Softener LLS | 2       | 2   | 2   | 2   | 2   | 2   | 2   | 2   |
| Catalyst 43          | ½       | ½   | ½   | ½   | ½   | ½   | ½   | ½   |
| Tear Strength:       |         |     |     |     |     |     |     |     |
| Warp                 | 0.8     | 0.9 | 1.0 | 1.1 | 0.8 | 0.9 | 0.9 | 0.9 |
| Fill                 | 0.9     | 0.9 | 1.1 | 1.2 | 0.8 | 0.9 | 0.9 | 0.9 |
| Crease Resistance:   |         |     |     |     |     |     |     |     |
| (W+F), Dry           | 314     | 304 | 291 | 282 | 317 | 304 | 301 | 293 |
| (W+F), Wet           | 284     | 297 | 273 | 276 | 293 | 296 | 293 | 284 |
| Stoll Flex Abrasion: |         |     |     |     |     |     |     |     |
| Warp                 | 24      | 37  | 100 | 199 | 29  | 79  | 102 | 131 |
| Fill                 | 81      | 74  | 157 | 206 | 44  | 90  | 101 | 123 |

TABLE 10

Fabric: 100% Cotton Broadcloth; Pretreatment: 25% Resin HK, 4.5% Catalyst 43, Dry at 200° F. for 3 minutes; Cure at 320° F. for 10 minutes.

|                      | Example |     |     |     |     |     |     |     |     |   |
|----------------------|---------|-----|-----|-----|-----|-----|-----|-----|-----|---|
|                      | 61      | 62  | 63  | 64  | 65  | 66  | 67  | 68  | 69  |   |
| NaCl                 | 25      | 25  | 25  | 25  | 20  | 20  | 20  | 20  | 20  | X |
| HCl                  | 3       | 3   | 3   | 3   | 3   | 3   | 3   | 3   | 3   | X |
| Temp., °F.           | 170     | 170 | 170 | 170 | 170 | 170 | 170 | 170 | 170 | X |
| Time (min.)          | 1       | 2   | 3   | 5   | 1   | 2   | 3   | 5   | 5   | X |
| Aftertreatment:      |         |     |     |     |     |     |     |     |     |   |
| Rhoplex K-3          | 3       | 3   | 3   | 3   | 3   | 3   | 3   | 3   | 3   |   |
| Bi-Chem Softener LLS | 2       | 2   | 2   | 2   | 2   | 2   | 2   | 2   | 2   |   |
| Catalyst 43          | ½       | ½   | ½   | ½   | ½   | ½   | ½   | ½   | ½   |   |
| Tear Strength:       |         |     |     |     |     |     |     |     |     |   |
| Warp                 | 1.0     | 0.9 | 0.9 | 0.9 | 0.9 | 1.0 | 0.9 | 0.9 | 0.6 |   |
| Fill                 | 1.0     | 1.0 | 0.9 | 0.9 | 0.8 | 1.0 | 0.9 | 0.9 | 0.6 |   |
| Crease Resistance:   |         |     |     |     |     |     |     |     |     |   |
| (W+F), Dry           | 283     | 271 | 265 | 256 | 298 | 275 | 271 | 254 | 326 |   |
| (W+F), Wet           | 278     | 270 | 266 | 252 | 283 | 268 | 276 | 268 | 304 |   |
| Stoll Flex Abrasion: |         |     |     |     |     |     |     |     |     |   |
| Warp                 | 140     | 223 | 194 | 202 | 97  | 275 | 173 | 205 | 13  |   |
| Fill                 | 226     | 135 | 129 | 146 | 96  | 91  | 139 | 200 | 21  |   |

TABLE 11

Fabric: 100% Cotton Broadcloth (4.20 oz./sq. yd.); Pretreatment: 25% Resin 183, 4.5% Catalyst 43, 3.0% Acrylic K-3, Dry 3 minutes at 200° F.; Cure 10 minutes at 320° F.

|                      | Example |     |     |     |     |     |     |     |     |     |
|----------------------|---------|-----|-----|-----|-----|-----|-----|-----|-----|-----|
|                      | 70      | 71  | 72  | 73  | 74  | 75  | 76  | 77  | 78  | 79  |
| Pre-Wet              | Yes     | Yes | Yes | Yes | Yes | Yes | Yes | Yes | X   | X   |
| NaCl                 | 15      | 15  | 20  | 20  | 20  | 20  | 20  | 20  | X   | X   |
| HCl                  | 5       | 5   | 3   | 3   | 3   | 3   | 3   | 3   | X   | X   |
| Temp., °F.           | 140     | 140 | 140 | 140 | 140 | 140 | 140 | 140 | X   | X   |
| Time (min.)          | 3       | 1   | 1   | 1   | 2   | 2   | 3   | 3   | X   | X   |
| Aftertreatment:      |         |     |     |     |     |     |     |     |     |     |
| Rhoplex K-3          | 1       | 1   | 1   | 1   | 1   | 1   | 1   | 1   | 1   | X   |
| Bi-Chem Softener PE  |         |     |     |     |     |     |     |     |     |     |
| Conc.                | 2       | 2   | 2   | 2   | 2   | 2   | 2   | 2   | 2   | X   |
| Catalyst 43          | ½       | ½   | ½   | ½   | ½   | ½   | ½   | ½   | ½   |     |
| Tear Strength:       |         |     |     |     |     |     |     |     |     |     |
| Warp                 | 2.9     | 2.7 | 2.7 | 2.6 | 2.9 | 3.0 | 2.7 | 2.8 | 2.4 | 2.3 |
| Fill                 | 2.5     | 2.6 | 2.7 | 2.5 | 2.6 | 2.8 | 2.7 | 2.7 | 2.4 | 2.3 |
| Crease Resistance:   |         |     |     |     |     |     |     |     |     |     |
| (W+F), Dry           | 308     | 317 | 317 | 305 | 283 | 293 | 299 | 299 | 311 | 314 |
| (W+F), Wet           | 293     | 298 | 301 | 277 | 261 | 273 | 285 | 305 | 305 | 278 |
| Stoll Flex Abrasion: |         |     |     |     |     |     |     |     |     |     |
| Warp                 | 176     | 55  | 115 | 392 | 525 | 122 | 181 | 271 | 16  | 31  |
| Fill                 | 152     | 64  | 86  | 282 | 243 | 306 | 106 | 180 | 35  | 52  |

<sup>1</sup> A polyethylene emulsion, manufactured by Bi-Chem Company, Division of Burlington Industries.

Table 12

Fabric: 65% Dacron/35% Cotton Cross Dyed; Pretreatment: 30% Resin 183, 5.5% Catalyst 43, 2% Rhoplex K-3, Dry 200° F. for 3 minutes; Cure 320° F. for 10 minutes.

|                           | Example |     |     |     |     |     |
|---------------------------|---------|-----|-----|-----|-----|-----|
|                           | 80      | 81  | 82  | 83  | 84  | 85  |
| Pre-Wet                   |         |     |     | Yes | X   | X   |
| NaCl                      | 20      | 20  | 20  | 20  | X   | X   |
| HCl                       | 3       | 3   | 3   | 3   | X   | X   |
| Temp., °F.                | 140     | 140 | 140 | 170 | X   | X   |
| Time (min.)               | 1       | 2   | 3   | ½   | X   | X   |
| Aftertreatment:           |         |     |     |     |     |     |
| Rhoplex K-3               | 2       | 2   | 2   | 2   | X   | 2   |
| Bi-Chem Softener PE Conc. | 2       | 2   | 2   | 2   | X   | 2   |
| Crystal 43                | ½       | ½   | ½   | ½   | X   | ½   |
| Tear Strength:            |         |     |     |     |     |     |
| Warp                      | 7.5     | 7.7 | 7.5 | 7.6 | 5.5 | 7.6 |
| Fill                      | 5.4     | 5.9 | 5.9 | 5.9 | 3.4 | 5.0 |
| Crease Resistance:        |         |     |     |     |     |     |
| (W+F), Dry                | 323     | 320 | 322 | 322 | 322 | 328 |
| (W+F), Wet                | 315     | 307 | 316 | 306 | 303 | 312 |
| Press Abrasion (Class)    | 3       | 3   | 4   | 3   | 1   | 2   |

TABLE 13.—EFFECT OF ALKALINE EARTH METAL ELECTROLYTE SALTS

Fabric: 100% Cotton, Army Twill, 8.0 oz./sq. yd.; Pretreatment: 25% Resin 183, 4.5% Catalyst 43, 5% Rhoplex K-3, Dry 200° F. for 3 minutes; Cure 320° F. for 10 minutes

|                                     | Example |     |     |        |        |     |       |     |       |       |
|-------------------------------------|---------|-----|-----|--------|--------|-----|-------|-----|-------|-------|
|                                     | 86      | 87  | 88  | 89     | 90     | 91  | 92    | 93  | 94    | 95    |
| CaCl <sub>2</sub> (anhydrous)       | 10      | 20  | 30  | 40     | 50     | 0   | 0     | 0   | 0     | 0     |
| MgCl <sub>2</sub> 6H <sub>2</sub> O | 0       | 0   | 0   | 0      | 0      | 10  | 20    | 30  | 40    | ----- |
| HCl (36%)                           | 3       | 3   | 3   | 3      | 3      | 3   | 3     | 3   | 3     | 3     |
| Time (min.)                         | 1       | 1   | 1   | 1      | 1      | 1   | 1     | 1   | 1     | 1     |
| Temperature, ° F.                   | 140     | 140 | 140 | 140    | 140    | 140 | 140   | 140 | 140   | ----- |
| Aftertreatment: <sup>1</sup>        |         |     |     |        |        |     |       |     |       |       |
| Rhoplex K-3                         | 5       | 5   | 5   | 5      | 5      | 5   | 5     | 5   | 5     | 2     |
| Bi-Chem Softener PE conc.           | 2       | 2   | 2   | 2      | 2      | 2   | 2     | 2   | 2     | 5     |
| Ammonium Chloride                   | 1/4     | 1/4 | 1/4 | 1/4    | 1/4    | 1/4 | 1/4   | 1/4 | 1/4   | 1/4   |
| Tear Strength:                      |         |     |     |        |        |     |       |     |       |       |
| Warp                                | 3.2     | 3.5 | 3.4 | 4.0    | 3.8    | 3.5 | 3.5   | 3.5 | 3.8   | 3.9   |
| Fill                                | 3.4     | 3.4 | 3.3 | 4.6    | 3.6    | 3.6 | 3.5   | 3.7 | 4.2   | 4.1   |
| Crease Resistance:                  |         |     |     |        |        |     |       |     |       |       |
| (W+F), Dry                          | 313     | 309 | 311 | 299    | 306    | 312 | 302   | 300 | 287   | 315   |
| (W+F), Wet                          | 300     | 299 | 301 | 294    | 311    | 302 | 300   | 300 | 296   | 290   |
| Stoll-Flex Abrasion:                |         |     |     |        |        |     |       |     |       |       |
| Warp                                | 257     | 248 | 277 | 532    | 296    | 351 | 454   | 343 | 537   | 370   |
| Fill                                | 1,118   | 738 | 763 | 1,500+ | 1,500+ | 631 | 1,056 | 815 | 1,034 | 1,315 |

<sup>1</sup> Dried 3 minutes at 200° F. and cured 3 minutes at 325° F.

TABLE 14.—EFFECT OF AMMONIUM CATION AND NITRATE ANION

Fabric: 100% Cotton, Army Twill, 8.0 oz./sq. yd.; Pretreatment: 25% Resin 183, 4.0% Catalyst 43, 5% Rhoplex K-3, Dry 200° F. for 3 minutes; Cure 320° F. for 10 minutes.

|                              | Example |     |       |       |       |       |
|------------------------------|---------|-----|-------|-------|-------|-------|
|                              | 96      | 97  | 98    | 99    | 100   | 101   |
| Sodium Nitrate               | 30      | 30  | ----- | ----- | ----- | ----- |
| Ammonium Chloride            |         |     | 25    | 25    | ----- | ----- |
| Potassium Nitrate            |         |     |       | 30    | 30    | ----- |
| Nitric Acid (70%)            | 3       | 3   | ----- | 3     | 3     | 3     |
| Hydrochloric Acid (36%)      |         |     | 3     | 3     | ----- | ----- |
| Time (min.)                  | 1       | 2   | 1     | 2     | 1     | 2     |
| Temperature, ° F.            | 140     | 140 | 140   | 140   | 140   | 140   |
| Aftertreatment: <sup>1</sup> |         |     |       |       |       |       |
| Rhoplex K-3                  | 5       | 5   | 5     | 5     | 5     | 5     |
| Bi-Chem Softener PE conc.    | 2       | 2   | 2     | 2     | 2     | 2     |
| Ammonium Chloride            | 1/4     | 1/4 | 1/4   | 1/4   | 1/4   | 1/4   |
| Tear Strength:               |         |     |       |       |       |       |
| Warp                         | 3.3     | 2.8 | 2.6   | 3.0   | 5.1   | 5.4   |
| Fill                         | 3.9     | 3.0 | 2.6   | 3.1   | 5.1   | 5.6   |
| Crease Resistance:           |         |     |       |       |       |       |
| (W+F), Dry                   | 297     | 297 | 312   | 298   | 306   | 296   |
| (W+F), Wet                   | 294     | 288 | 304   | 290   | 300   | 296   |
| Stoll-Flex Abrasion:         |         |     |       |       |       |       |
| Warp                         | 763     | 599 | 647   | 593   | 408   | 767   |
| Fill                         | 1,681   | 997 | 1,120 | 656   | 651   | 1,028 |

<sup>1</sup> Dried 3 minutes at 200° F. and cured 3 minutes at 325° F.

### EXAMPLE 102

This example relates to an illustration of the improved moisture regain obtained by the present invention. The textile product of Example 53 was tested for moisture regain, according to ASTM Test D629-59A, and compared with the resinated control textile of Example 69. The test results were as follows:

| Moisture regain                       | Percent |
|---------------------------------------|---------|
| Resinated control (of Ex. 69)         | 3.4     |
| Resinated acid hydrolysis (of Ex. 53) | 4.9     |
| Percent improvement                   | 44      |

### EXAMPLE 103

This example relates to an illustration of the improved soil resistance of the textiles of the present invention. The textile produced according of Example 82 was tested for soil resistance by the 3-M Test and compared with the resinated control textile of Example 85. The test produced the following results:

| Reflectance                            | Percent |
|----------------------------------------|---------|
| Resinated control (of Ex. 85):         |         |
| Original                               | 99.6    |
| Tested                                 | 57.7    |
| Resinated acid hydrolysis (of Ex. 62): |         |
| Original                               | 112.5   |
| Tested                                 | 77.7    |
| Percent improvement                    | 34.6    |

Obviously many modifications and variations of the present invention are possible in the light of the above teachings. It is therefore to be understood that within 50 the scope of the appended claims the invention may be practiced otherwise than as specifically described.

What we claim is:

- In a process of producing resin-treated cellulosic textiles comprising applying a resin to a cellulosic textile, and at least partially curing the resin on the textile by means of a cross-linking agent, the improvement comprising (a) hydrolyzing the partially cured resin-treated textile in an aqueous bath containing a strong acid and a neutral or only slightly acid electrolyte salt 60 selected from the group consisting of alkali metal, alkaline earth metal and ammonium salt electrolytes, the concentration of the electrolyte salt being at least 5% w/v. and the concentration of the acid being 0.01 to 15% w/v., and (b) thereafter neutralizing and washing the hydrolyzed resin-treated textile, whereby the textile has increased abrasion resistance and other improved textile properties.
- The process as claimed in claim 1 wherein the electrolytic salt is a salt of said acid.
- The process as claimed in claim 1 wherein 0.1 to 30 percent by weight of an acrylic resin and 0.1 to 10 percent by weight of a lubricating agent are applied to the resin-treated cellulose textile.
- The process as claimed in claim 3 wherein said acrylic resin and said lubricating agent are applied to the

resin-treated cellulose textile before and after the hydrolyzing step.

5. The process as claimed in claim 1 wherein the resin-treated cellulose textile is pre-wetted prior to the hydrolyzing step.

6. The process as claimed in claim 1 wherein the hydrolyzed resin-treated textile is neutralized by immersion in an aqueous bath containing a weak alkaline compound.

7. The process as claimed in claim 6 wherein the concentration of the weak alkaline compound in the neutralized bath is 0.01 to 10 percent w./v.

8. The process of claim 1 wherein the acid is hydrochloric acid, the salt is sodium chloride and the hydrolyzed resin-treated textile is neutralized by impregnating same with an aqueous solution of sodium carbonate, followed by washing with water and drying.

10

15

## UNITED STATES PATENTS

|             |         |               |             |
|-------------|---------|---------------|-------------|
| 2,536,050   | 1/1951  | Fluck         | 117-143 X   |
| 2,823,142   | 2/1958  | Sumner et al. | 117-140 X   |
| 5 2,950,553 | 8/1960  | Hurwitz       | 117-139.4 X |
| 2,957,746   | 10/1960 | Buck et al.   | 117-139.4 X |
| 2,993,746   | 7/1961  | Miles et al.  | 117-62.1 X  |
| 3,004,868   | 10/1961 | Sumner et al. | 117-140     |
| 3,009,832   | 11/1961 | Burkitt       |             |
| 3,138,802   | 6/1964  | Getchell      | 117-139.4 X |
| 3,374,107   | 3/1968  | Cotton        | 117-139.4   |

WILLIAM D. MARTIN, Primary Examiner

15 H. J. GWINNELL, Assistant Examiner

U.S. Cl. X.R.

117-139.4, 139.5, 143, 145